

## UNITED STATES PATENT OFFICE

GEOORG MASING, OF BERLIN, AND OTTO DAHL, OF BERLIN-CHARLOTTENBURG, GERMANY, ASSIGNORS TO SIEMENS & HALSKE, AKTIENGESELLSCHAFT, OF SIEMENS-STADT, NEAR BERLIN, GERMANY, A CORPORATION OF GERMANY

## PROCESS FOR THE IMPROVEMENT OF THE PROPERTIES OF IRON-BERYLLIUM ALLOYS

No Drawing. Application filed April 5, 1928, Serial No. 267,796, and in Germany April 12, 1927.

The present invention relates to a new and useful process for the improvement of the properties of iron-beryllium alloys. More particularly, the hardness or the strength and toughness of the iron-beryllium alloy can be brought to very favourable values by using the new process.

According to the invention the iron-beryllium alloys are subjected to a suitable heat treatment. To that end the alloy can be sufficiently quickly cooled in air or by quenching for instance from temperatures above 550° C. and up to about 1200° C. and, if desired, submitted to a second heating to a lower temperature of about 250 to 500° C. In an alloy with a beryllium proportion of about 4%, a hardness of approximately 600 Brinell was obtained by the process described, whilst the hardness after the quenching and before the second heating amounted to about 320 Brinell.

The process according to the invention is also applicable with success for iron-beryllium alloys which contain up to about 40% of one or more other elements such as aluminium, nickel, copper, tin, zinc, cadmium, cobalt or some percents of carbon or silicium. Sometimes it is advisable to combine the thermic treatment with a preliminary mechanical working, as for instance hammering or rolling. The improvement of the properties takes place in the case of cast alloys as well as of rolled alloys of the kind mentioned. The beryllium percentage preferably lies below 13.

What we claim as our invention and desire to be secured by Letters Patent is:

1. A method of increasing the hardness, strength and tenacity of iron-beryllium alloys having a beryllium content of not greater than thirteen percent, which comprises heating such alloys to a temperature of at least 550° C. and then quickly cooling said alloys.

2. A method of increasing the hardness, strength and tenacity of iron-beryllium alloys having a beryllium content of not greater than thirteen percent, which comprises heating such alloys to a temperature of at least 550° C., quickly cooling said al-

loys and then re-heating said alloys to a lower temperature.

3. A method of increasing the hardness, strength and tenacity of iron-beryllium alloys having a beryllium content of not greater than thirteen percent, which comprises heating such alloys to a temperature of at least 550° C., quickly cooling said alloys, and then re-heating said alloys to a temperature between 250° and 350° C.

4. A method of increasing the hardness, strength and tenacity of alloys containing iron, up to 13% of beryllium and up to 40% of a metal selected from the group comprising aluminum, nickel, copper, tin, zinc, cadmium and cobalt, which comprises heating said alloys to a temperature of at least 550° C., quickly cooling the same, and then re-heating said alloys to a lower temperature.

In testimony whereof we affix our signatures.

GEORG MASING.  
OTTO DAHL.

75

80

85

90

95

100